

Aug. 28, 1951

B. H. CARROLL ET AL  
PHOTOGRAPHIC SILVER HALIDE EMULSION SUPERSENSITIZED  
WITH A BENZIMIDAZOLE BASE  
Filed April 20, 1946

2,566,167

Fig. 1.



A = 3,3'-diethyl-9-methylselenacarbocyanine bromide.

B = 3,3'-diethyl-9-methylselenacarbocyanine bromide  
plus benzimidazole.

Fig. 2



C = 3,3'-diethyl-9-methylselenacarbocyanine bromide.

D = 3,3'-diethyl-9-methylselenacarbocyanine bromide  
plus 2-methylbenzimidazole.

BURT H. CARROLL  
JOHN SPENCE  
INVENTORS

BY *R. M. Perrino*  
*Daniel J. Mayne*  
ATTORNEYS

## UNITED STATES PATENT OFFICE

2,566,167

PHOTOGRAPHIC SILVER HALIDE EMULSION  
SUPERSENSITIZED WITH A BENZIMIDA-  
ZOLE BASEBurt H. Carroll and John Spence, Rochester,  
N. Y., assignors to Eastman Kodak Company,  
Rochester, N. Y., a corporation of New Jersey

Application April 20, 1946, Serial No. 663,763

10 Claims. (Cl. 95—7)

**1** This invention relates to sensitized photographic emulsions and to a process for preparing the same. This application is a continuation-in-part of our copending application Serial No. 466,796, filed November 24, 1942 (now United States Patent 2,398,778, dated April 23, 1946).

It is known that the spectral distribution of spectral sensitivity of certain spectrally sensitized emulsions can be altered and an increase of sensitivity obtained in some spectral region, by incorporating certain additional sensitizing dyes in the spectrally sensitized emulsions. (See United States Patent 2,158,882, dated May 16, 1939, and 2,159,565, dated May 23, 1939.) The effect thus produced has come to be known as supersensitization. Supersensitization of certain spectrally sensitized emulsions can also be effected by incorporating certain substantially colorless heterocyclic bases, viz. those containing an amino group, in the spectrally sensitized emulsions. (See United States Patent 2,177,635, dated October 31, 1939.) Supersensitization differs from hypersensitization which involves treatment of finished films or plates, an operation which normally reduces the pAg and increases the pH of the emulsion, with consequent decreased stability.

We have now found a new method for supersensitizing spectrally sensitized emulsions, which not only does not reduce the stability of the emulsions, but is especially valuable as a means of giving good panchromatic sensitized emulsions of high speed and good color balance.

**30** It is, accordingly, an object of our invention to provide new supersensitized photographic emulsions. A further object is to provide a process for preparing such emulsions. Other objects will become apparent hereinafter.

In accordance with the invention, a photographic silver halide emulsion other than a chloride emulsion, e. g. silver chlorobromide (which may contain small amounts of silver iodide), silver bromide or silver bromiodide emulsions, spectrally sensitized with a (at least one) cyanine dye is supersensitized by incorporating in the emulsion one or more benzimidazole bases. Our invention is directed principally to emulsions of such grain size that the emulsions give a substantially neutral-toned image in Eastman Kodak Company's "D-76" developer, and should not be confused with prior proposals to obtain blue-black tones in fine-grain emulsions by means of heterocyclic nitrogen bases. Moreover, our invention involves incorporation of the benzimidazole bases in the emulsion before exposure of the emulsion and should not be confused with

proposals to develop with color-forming developers silver salt images, in the presence of certain heterocyclic nitrogen bases which contain a reactive methyl group.

**5** The benzimidazole bases advantageously employed in practicing our invention are of a specific type and can be defined as benzimidazole (benzimidazoles) bases selected from the group consisting of benzimidazole and benzimidazole containing a substituent (i. e. at least one substituent) selected from the group consisting of alkyl groups, alkoxy groups, hydroxyalkyl groups, aryl groups, aryloxyl groups, alkylmercapto groups, arylmercapto groups, acyl groups, acyloxyl groups and halogen atoms. Examples of such substituents are: methyl, ethyl, methoxyl, ethoxyl, hydroxyethyl, phenyl, phenoxy, methylmercapto, ethylmercapto, phenylmercapto, acetyl, propionyl, benzoyl, acetoxy (acetoxy), propionoxyl (propionoxy) and benzoxy groups, and chlorine, bromine and iodine atoms.

**10** Exemplary of the benzimidazole bases advantageously employed in practicing our invention are benzimidazole which has the following formula:



1-acetylbenzimidazole  
1-methylbenzimidazole  
2-methylbenzimidazole  
4-methylbenzimidazole  
5-methylbenzimidazole  
1-phenylbenzimidazole  
2-phenylbenzimidazole  
5-methoxybenzimidazole, etc.

**15** The majority of cyanine dyes which are supersensitized by the benzimidazole bases are characterized by the fact that the dyes produce two types of sensitization depending upon conditions. Such different types of sensitization are described by Leermakers, Carroll and Staud, J. Chem. Physics 5, 878 (1937), and by Schwarz, Sci. et Ind. Phot. 10, 233 (1939). When a cyanine dye of this type is used as a sensitizer in low concentration, it exhibits a sensitizing maximum displaced about 20 to 50 mu. toward the red from the absorption maximum in ethyl alcohol solution. On increasing the concentration of the dye, or upon digesting the emulsion containing the dye in the lower concentration, or both, a second maximum of sensitization develops at longer wavelengths, which may be accompanied by an

increase in total optical sensitization. In some cases, a decrease in sensitivity at the first maximum can be detected. These phenomena are consistent with the hypothesis of two states of the sensitizing dye in an equilibrium which is controlled by concentration. The benzimidazole bases favor the formation of a second maximum which occasionally is appreciably displaced from the normal second maximum. The increase in sensitivity apparently corresponds to increased conversion of the dye to the state corresponding to the second maximum of sensitization. In some cases, the effect appears to correspond to a more complete conversion than has ever been obtained without a supersensitizer, and in any case the long wavelength sensitivity is better than can be obtained from the same concentration of dye without the benzimidazole base.

The following are exemplary of the cyanine dyes which are supersensitized in accordance with our invention:

3,1'-diethyl-6'-methoxy-2'-cyanine iodide.  
 3,3'-diethyl-9-methylthiacyanine bromide.  
 9-ethyl-3,3'-dimethylthiacyanine bromide.  
 5'-chloro-3,3',9-triethylthiacyanine iodide.  
 5,5'-dichloro-3,3',9-triethylthiacyanine iodide.  
 3,3'-diethyl-9-methyl-4,5,4',5'-dibenzothiacyanine bromide.  
 3,3'-diethyl-9-methylselenathiacyanine bromide.  
 5'-chloro-3,3'-diethyl-9-methylselenathiacyanine iodide.  
 3,3'-diethyl-9-methylselenacyanine bromide.  
 1'-ethyl-3,6'-dimethyl-4-phenylthiazolo-2'-cyanine bromide.  
 3,1'-diethyl-6'-methoxythia-2'-cyanine bromide.  
 1,1'-diethyl-2,2'-cyanine bromide.  
 1,1'-diethyl-2,2'-carbocyanine bromide.  
 9-ethyl-3,1'-dimethylthia-2'-carbocyanine iodide.  
 3,3'-diethyl-9-methyl-5-phenyloxathiacyanine iodide.  
 3,3'-diethyloxatricarbocyanine iodide.

The sensitizing dyes can be employed in any desired concentration. Ordinarily from 10 to 30 mg. of dye per liter of emulsion will suffice to produce the optimum sensitizing effect. The methods of incorporating sensitizing dyes in emulsions are well known to those skilled in the art. Ordinarily it is preferable to dissolve the dye in a water-miscible solvent, such as methanol or ethanol, before incorporating in the emulsion. One or more sensitizing dyes can be employed.

The amount of benzimidazole base employed is not critical. Usually the full supersensitizing effect is developed at a concentration of 0.10 to 1.5 grams per liter of emulsion. At these concentrations practically none of the benzimidazole bases has an appreciable effect on the pH of the emulsion. The benzimidazole bases can be added to the emulsions with, before or after the sensitizing dye or dyes. More than one benzimidazole base can be employed. The benzimidazole bases are preferably, but not necessarily, diluted with a water-miscible solvent, such as methanol, before incorporation in the emulsions. The sensitizing dye or dyes and the benzimidazole base or bases can be added to the emulsions at any convenient stage of their preparation, but preferably to the washed, finished emulsions before coating.

The following examples will serve to illustrate further the results obtained in accordance with our invention.

#### Example 1

A slow negative gelatino-silver-chlorobromide developing-out emulsion was sensitized with 3,3'-diethyl-9-methylselenacyanine bromide (20 mg. per liter of emulsion) and to a portion of the spectrally sensitized emulsion was added benzimidazole ( $C_7H_6N_2$ ). A portion of the spectrally sensitized emulsion without the benzimidazole, and the portion containing it were exposed through red (Wratten No. 25) and minus blue (Wratten No. 12) filters. The results are tabulated below.

| benzimidazole<br>(g. per liter of<br>emulsion) | Red   |       | Minus Blue |       |
|------------------------------------------------|-------|-------|------------|-------|
|                                                | Speed | Gamma | Speed      | Gamma |
| none                                           | 10.6  | 3.91  | 29.0       | 3.65  |
| 0.58                                           | 16.5  | 3.91  | 43.5       | 4.40  |

#### Example 2

A fast negative gelatino-silver-bromide developing-out emulsion was sensitized with 3,3'-diethyl-9-methylselenacyanine bromide (20 mg. per liter of emulsion) and to a portion of the spectrally sensitized emulsion was added 2-methylbenzimidazole. A portion of the spectrally sensitized emulsion without the 2-methylbenzimidazole and a portion containing it were exposed through red (Wratten No. 25) and minus blue (Wratten No. 12) filters. The results are tabulated below:

| 2-methylbenzi-<br>midazole<br>(g. per liter of<br>emulsion) | Red   |       | Minus Blue |       |
|-------------------------------------------------------------|-------|-------|------------|-------|
|                                                             | Speed | Gamma | Speed      | Gamma |
| none                                                        | 120   | 1.42  | 600        | 1.51  |
| 0.25                                                        | 290   | 1.26  | 800        | 1.47  |

Some of the benzimidazole bases, while effecting an increase of sensitivity (speed) in some spectral region, cause a decrease in others, and must be employed with that fact in mind.

The accompanying drawing illustrates graphically the supersensitizing effect obtained with two of our new combinations in a gelatino-silver-bromide emulsion. Each figure in the drawing is a diagrammatic reproduction of two spectrograms. In Fig. 1, Curve A represents the sensitivity of a gelatino-silver-bromide emulsion containing 3,3'-diethyl-9-methylselenacyanine bromide in a concentration of 20 mg. per liter of emulsion. Curve B represents the sensitivity of the same emulsion containing 3,3'-diethyl-9-methylselenacyanine bromide in a concentration of about 20 mg. per liter of emulsion and containing, in addition, benzimidazole in a concentration of about 0.58 g. per liter of emulsion. It will be observed that with the benzimidazole in the emulsion, a new sharp maximum appears at about 640  $m\mu$  and the red speed is considerably increased. In Fig. 2, Curve C represents the sensitivity of a gelatino-silver-bromide emulsion containing 3,3'-diethyl-9-methylselenacyanine bromide in a concentration of 20 mg. per liter of emulsion. Curve D represents the sensitivity of the same emulsion containing 3,3'-diethyl-9-methylselenacyanine bromide in a concentration of about 20 mg. per liter of emulsion and containing, in addition, 2-methylbenzimidazole in a concentration of about 0.25 g. per liter of emulsion. It will be observed that the maximum of sensitivity is shifted to about 610  $m\mu$ .

Our invention is primarily directed to the customarily employed gelatino-silver-halide developing-out emulsions, such as gelatino-silver-chlorobromide, gelatino-silver-bromide and gelatino-silver-bromiodide developing-out emulsions, especially emulsions for development to black-and-white images by means of non-color-forming developers, e. g. hydroquinone-N-methyl-p-amino-phenol developers.

Emulsions prepared in accordance with our invention can be coated in the usual manner upon any desired support, such as cellulose nitrate support, cellulose acetate support, polyvinyl acetal resin support, metal support, glass support or paper support.

Cyanine dyes are described and defined, e. g. in "The Theory of the Photographic Process," by C. E. K. Mees, The MacMillan Company, New York, 1942.

What we claim as our invention and desire to be secured by Letters Patent of the United States is:

1. A photographic silver halide emulsion selected from the group consisting of silver chlorobromide, silver bromide and silver bromiodide developing-out emulsions spectrally sensitized with a sensitizing cyanine dye and containing, as a supersensitizer, a benzimidazole base selected from the group consisting of benzimidazole and benzimidazole containing a substituent selected from the group consisting of halogen atoms, alkyl groups, alkoxy groups, hydroxyalkyl groups, aryl groups containing only carbon and hydrogen atoms, aryloxy groups in which the aryl portion contains only carbon and hydrogen atoms, alkylmercapto groups, arylmercapto groups in which the aryl portion contains only carbon and hydrogen atoms, acyl groups containing only carbon and hydrogen atoms plus one oxygen atom, and acyloxy groups containing only carbon and hydrogen atoms plus two oxygen atoms.

2. A photographic gelatino-silver-halide developing-out emulsion selected from the group consisting of silver chlorobromide, silver bromide and silver bromiodide developing-out emulsions spectrally sensitized with a sensitizing cyanine dye and containing, as a supersensitizer, a benzimidazole base selected from the group consisting of benzimidazole and benzimidazole containing a substituent selected from the group consisting of halogen atoms, alkyl groups, alkoxy groups, hydroxyalkyl groups, aryl groups containing only carbon and hydrogen atoms, aryloxy groups in which the aryl portion contains only carbon and hydrogen atoms, alkylmercapto groups, arylmercapto groups in which the aryl portion contains only carbon and hydrogen atoms, acyl groups containing only carbon and hydrogen atoms plus one oxygen atom, and acyloxy groups containing only carbon and hydrogen atoms plus two oxygen atoms.

3. A photographic gelatino-silver-halide developing-out emulsion selected from the group consisting of silver chlorobromide, silver bromide and silver bromiodide developing-out emulsions spectrally sensitized with a sensitizing cyanine dye and containing, as a supersensitizer, 2-methylbenzimidazole which has the formula:



4. A photographic gelatino-silver-halide developing-out emulsion selected from the group consisting of silver chlorobromide, silver bromide and silver bromiodide developing-out emulsions spectrally sensitized with a sensitizing cyanine dye which produces a maximum of spectral sensitivity in the emulsion at one concentration and at a higher concentration, or upon digestion of the emulsion containing the dye at the lower concentration, produces a second maximum of sensitivity at a wavelength longer than that of the first maximum, the emulsion containing, as a supersensitizer, a benzimidazole base selected from the group consisting of benzimidazole and benzimidazole containing a substituent selected from the group consisting of halogen atoms, alkyl groups, alkoxy groups, hydroxyalkyl groups, aryl groups containing only carbon and hydrogen atoms, aryloxy groups in which the aryl portion contains only carbon and hydrogen atoms, alkylmercapto groups, arylmercapto groups in which the aryl portion contains only carbon and hydrogen atoms, acyl groups containing only carbon and hydrogen atoms plus one oxygen atom, and acyloxy groups containing only carbon and hydrogen atoms plus two oxygen atoms.

5. A photographic gelatino-silver-halide developing-out emulsion selected from the group consisting of silver chlorobromide, silver bromide and silver bromiodide developing-out emulsions spectrally sensitized with a sensitizing cyanine dye which produces a maximum of spectral sensitivity in the emulsion at one concentration and at a higher concentration, or upon digestion of the emulsion containing the dye at the lower concentration, produces a maximum of sensitivity at a wavelength longer than that of the first maximum, the emulsion containing, as a supersensitizer, benzimidazole having the formula:



6. A photographic gelatino-silver-bromiodide developing-out emulsion spectrally sensitized with a sensitizing cyanine dye which produces a maximum of spectral sensitivity in the emulsion at one concentration and at a higher concentration, or upon digestion of the emulsion containing the dye at the lower concentration produces a maximum of sensitivity at a wavelength longer than that of the first maximum, the emulsion containing as a supersensitizer, a benzimidazole base selected from the group consisting of benzimidazole and benzimidazole containing a substituent selected from the group consisting of halogen atoms, alkyl groups, alkoxy groups, hydroxyalkyl groups, aryl groups containing only carbon and hydrogen atoms, aryloxy groups in which the aryl portion contains only carbon and hydrogen atoms, alkylmercapto groups, arylmercapto groups in which the aryl portion contains only carbon and hydrogen atoms, acyl groups containing only carbon and hydrogen atoms plus one oxygen atom, and acyloxy groups containing only carbon and hydrogen atoms plus two oxygen atoms.

7. A photographic gelatino-silver-bromiodide developing-out emulsion spectrally sensitized with a sensitizing dye which produces a maximum of spectral sensitivity in the emulsion at one concentration and at a higher concentration, or upon digestion of the emulsion containing the

dye at the lower concentration produces a maximum of sensitivity at a wavelength longer than that of the first maximum, the emulsion containing, as a supersensitizer, benzimidazole having the formula:



8. A photographic gelatino-silver-bromide developing-out emulsion spectrally sensitized with a sensitizing dye which produces a maximum of spectral sensitivity in the emulsion at one concentration and at a higher concentration, or upon digestion of the emulsion containing the dye at the lower concentration produces a maximum of sensitivity at a wavelength longer than that of the first maximum, the emulsion containing, as a supersensitizer, 2-methylbenzimidazole having the formula:



9. A photographic gelatino-silver-halide developing-out emulsion selected from the group consisting of silver chlorobromide, silver bromide and silver bromide developing-out emulsions spectrally sensitized with a sensitizing cyanine dye and containing, as a supersensitizer, benzimidazole which has the formula:



10. A photographic gelatino-silver-halide developing-out emulsion selected from the group consisting of silver chlorobromide, silver bromide and silver bromide developing-out emulsions spectrally sensitized with a sensitizing cyanine dye which produces a maximum of spectral sensitivity in the emulsion at one concentration and at a higher concentration, or upon digestion of the emulsion containing the dye at the lower concentration, produces a maximum of sensitivity at a wavelength longer than that of the first maximum, the emulsion containing, as a supersensitizer, 2-methylbenzimidazole having the formula:

15

20

35

40



BURT H. CARROLL,  
JOHN SPENCE.

#### REFERENCES CITED

The following references are of record in the file of this patent:

#### UNITED STATES PATENTS

| Number    | Name     | Date           |
|-----------|----------|----------------|
| 2,066,099 | Dieterle | Dec. 29, 1936  |
| 2,158,882 | Mees     | May 16, 1939   |
| 2,296,306 | Peterson | Sept. 22, 1942 |
| 2,353,754 | Peterson | July 18, 1944  |